

## 1

3,496,039

## EXPLOSIVE COMPOSITIONS CONTAINING AN AROMATIC NITRO COMPOUND AND CALCIUM PHOSPHATE

Adolf Berthman and Paul Lingens, Leverkusen, Germany, 5 assignors to Dynamit Nobel Aktiengesellschaft, a corporation of Germany  
No Drawing. Filed Nov. 29, 1968, Ser. No. 782,510  
Claims priority, application Germany, Nov. 29, 1967,

1,646,284

Int. Cl. C06b 9/00

U.S. Cl. 149—2

5 Claims

## ABSTRACT OF THE DISCLOSURE

In an explosive composition comprising fusible aromatic nitro compounds, the improvement which comprises calcium phosphate fume in a minor proportion effective to improve detonation characteristics, thermal stability or exudation characteristics. The calcium phosphate fume is characterized by low density and high specific surface area.

The invention relates to the improvement of the properties of explosives and explosive compositions of fusible aromatic compounds, particularly TNT and trinitrobenzene, or mixtures of these nitro compounds with nitramines and/or with nitric acid esters, e.g. mixtures with tetryl and/or nitropentaerythrol (nitropenta), including eutetics with tetryl or nitropenta, by adding finely divided calcium phosphate to them. Known additives, such as metal powders or desensitizers can be included.

The calcium phosphate has been manufactured by mixing phosphoric acid with the required amount of calcium nitrate or calcium chloride to form a clear solution or paste, and by spraying this mixture into a current of hot inert gas at temperatures of 190 to 450° C. The production of the calcium phosphate fume is described in DAS 1,196,166, issued to "Chemische Fabrik Kalk." We call this product calcium phosphate fume. The calcium phosphate fume is a finely divided product having a large specific surface area, in general about 10–50 m.<sup>2</sup>/g., and having an extremely low bulk density in general about 0.01–0.07 g./cm.<sup>3</sup>. It is added to the explosive components in minor proportion, e.g. a quantity of 0.1 to 15%, preferably 0.2 to 5% by weight of the composition.

It has been found that the addition of the above-mentioned calcium phosphates to the fusible aromatic nitro compositions and compounds, for example, TNT and trinitrobenzene, surprisingly modifies particularly the following three properties;

- (1) The capability of detonation is improved;
- (2) Thermal stability and shock resistance; and
- (3) The exudation of impurities is largely prevented.

Also particularly surprising was the extent to which the properties of the castable explosives according to the invention changed. This is made apparent hereinafter by a comparison between TNT charges with and without the addition of calcium phosphate.

## EXAMPLE 1

Sticks of TNT were cast with and without the addition of calcium phosphate. The length of the sticks was 20 cm., and the diameter was varied. The sticks of explosives were ignited with a pressed pellet of 15 g. of tetryl and were stood up on a lead plate which served as an indicator for complete detonation. The tests were performed without any enclosure. A stick of TNT having a diameter of 50 mm. and no additive would not propagate the detonation and the lead plate was undamaged.

## 2

If the TNT contained 1% calcium phosphate (specific surface area 15 m.<sup>2</sup>/g.; bulk density of 0.03 g./cm.<sup>3</sup>), the charge detonated perfectly all the way through the stick, even at a diameter of 10 mm.

Cast TNT cylinders 200 mm. long and 28 mm. in diameter and having a specific weight of 1.60 g./cm.<sup>3</sup> could not be detonated with No. 8 aluminum blasting caps. With the addition of 1.5% calcium phosphate, such explosive sticks detonated perfectly all the way through. 10 The density of this explosive composition according to the invention amounted to 1.58 g./cm.<sup>3</sup>. The tests were performed with any wrapper or enclosure. At the end of the stick opposite the blasting cap, a detonation speed of 6600 m./s. was measured. If 12 or 15% calcium phosphate was added to the molten TNT, a paste-like composition was obtained having a specific weight of 1.61 g./cm.<sup>3</sup> and 1.64 g./cm.<sup>3</sup>, respectively. Cylinders 200 mm. long and 28 mm. in diameter prepared from this composition could not be detonated, even with a No. 6 blasting cap containing 0.5 g. of PETN and 0.5 g. of potassium chloride as a booster. The detonation speed amounted to 6500 and 6200 m./s. respectively.

The advantage of the improved detonability consists mainly in the fact that TNT charges can be detonated easily without the use of boosters made of pressed tetryl, PETN, hexogen or TNT. In fact, cast TNT charges containing the calcium phosphate additive according to the invention can be used as boosters for explosives that are difficult to initiate. For example, slurries can be detonated in blasting holes with detonators made of TNT and the calcium phosphate additive according to the invention, instead of charges of cast pentolite such as are used today.

The improvement in thermal stability and shock resistance is clarified by the following experiments: 0.4 g. of TNT with and without the addition of calcium phosphate according to the invention was finely ground and placed in a glass test tube. This tube was placed in a heated bath of Woods' metal which was adjusted to a constant temperature. The time it took for the TNT to flash or explode was determined. The longer this time is, the better the explosion tolerates thermal stress. The time for TNT amounted to 38 seconds, and for TNT containing the addition of 2% calcium phosphate according to the invention amounted to 75 seconds. The falling weight impact tests were performed according to Koenen Ide (Explosivstoffe," No. 2, February 1961, pp. 34–36). With a weight of 5 kg. and a 10 cm. drop, the first explosions produced in the TNT were without additive. If the TNT contained the addition of 2% calcium phosphate according to the invention, the beginning of the reactions was not obtained until the drop amounted to 20 cm. The following results were measured for the total of 6 tests of each explosive at heights of 10, 20, 30, 40, 50 and 60 cm.:

|                       | TNT | 98 = TNT,<br>2 = calcium<br>phosphate |
|-----------------------|-----|---------------------------------------|
| No reaction.....      | 24  | 28                                    |
| Partial reaction..... | 0   | 4                                     |
| Explosion.....        | 12  | 4                                     |

The advantage of the addition of calcium phosphate according to the invention consists in the fact that, in spite of the significant improvement of detonability, safety against shock and heat increase.

When explosive bodies made of impure TNT are exposed for a relatively long time to a temperature of about 70° C., a eutectic mixture formed by the impurities with the TNT exudes. The TNT bodies were 40 mm. high and 21 mm. in diameter. They were placed on a filter

paper and exposed for 20 hours to a temperature of 70° C. This produced spots of greater or lesser size on the filter paper. The larger the diameter of these spots, the greater is the tendency of the explosive to exudation. For a TNT with a solidification point of 80.47° C., a spot diameter of 44 mm. was measured. If increasing amounts of calcium phosphate are added to this TNT, the following spot diameters are measured:

| Calcium phosphate content (percent): | spot diameter, mm. | 10 |
|--------------------------------------|--------------------|----|
| 0                                    | 44                 |    |
| 0.1                                  | 36                 |    |
| 0.5                                  | 19                 |    |
| 1                                    | 13.6               | 15 |
| 2                                    | 6.3                |    |

The advantage of the addition of calcium phosphate according to the invention consists, according to this experiment, in the fact that cast TNT charges can be stored at higher temperatures, e.g., in hot sunlight, without the occurrence of exudation.

#### EXAMPLE 2

The experimental results described in Example 1, involving explosive charges of TNT with and without the addition of calcium phosphate according to the invention were obtained in like manner also with explosive compositions made of aromatic nitro compounds and metal powders. A cast stick (200 mm. long, 28 mm. diam.) made of a mixture of 75% TNT and 25% aluminum powder with the addition of 2% calcium phosphate (specific surface area 15 m.<sup>2</sup>/g.; bulk density 0.03 g./cm.<sup>3</sup>) according to the invention could be detonated with a No. 8 aluminum blasting cap, for example, while the same mixture without the addition of the calcium phosphate could not be initiated with a No. 8 aluminum blasting cap. A mixture of 47.6% TNT and 52.4% aluminum required 59 seconds to flash or explode at a temperature of 340° C. However, if 1 part of calcium phosphate was added to the mixture, the time required to ignite it amounted to 67 seconds. The size of the spot produced by bleeding was measured at 38 mm. for the mixture of 75% TNT (solidification point 80.47° C.) and 25% aluminum. With the addition of 1% calcium phosphate according to the invention, the diameter of the spot amounted to only 11 mm.

#### EXAMPLE 3

In the case of explosive compositions containing a sufficient amount of nitramines or nitric acid esters, the improvement of detonatability by the addition of calcium phosphate according to the invention is of no importance. Consequently, it has not been our aim to bring about an improvement of the initiability of such compositions. In the case of such explosive mixtures, flashing or explosion was produced at 238° C. after the following periods—

| Mixture A:                                                                                                               |         |      |
|--------------------------------------------------------------------------------------------------------------------------|---------|------|
| 40% TNT (solidification point 80.47° C.),                                                                                |         |      |
| 60% hexogen                                                                                                              | seconds | 33   |
| Spot diameter                                                                                                            | mm      | 40   |
| Mixture B:                                                                                                               |         |      |
| 39% TNT (solidification point 80.47° C.),                                                                                |         |      |
| 60% hexogen, 1% calcium phosphate (specific surface area 12 m. <sup>2</sup> /g.; bulk density 0.07 g./cm. <sup>3</sup> ) | seconds | 40   |
| Spot diameter                                                                                                            | mm      | 10.5 |

#### EXAMPLE 4

In the case of explosive compositions of TNT (solidification point 80.47° C.), hexogen and powdered aluminum, flashing or explosion was produced at 235° C. within the periods specified below, the specific weights and spot diameters being also given—

#### Mixture A:

|                 |                     |      |
|-----------------|---------------------|------|
| TNT             | percent             | 35   |
| Hexogen         | do                  | 40   |
| Aluminum powder | do                  | 25   |
| Time            | seconds             | 30   |
| Spec. weight    | g./cm. <sup>3</sup> | 1.85 |
| Spot diameter   | mm                  | 35   |

#### Mixture B:

|                                                                                               |                     |      |
|-----------------------------------------------------------------------------------------------|---------------------|------|
| TNT                                                                                           | percent             | 30   |
| Hexogen                                                                                       | do                  | 40   |
| Aluminum powder                                                                               | do                  | 25   |
| Desensitizer consisting of 4.2 parts paraffin wax, 0.7 part nitrocellulose, 0.1 part lecithin | do                  | 5    |
| Time                                                                                          | seconds             | 29   |
| Specific weight                                                                               | g./cm. <sup>3</sup> | 1.77 |
| Spot diameter                                                                                 | mm                  | >50  |

#### Mixture C:

|                                                                                                       |                     |      |
|-------------------------------------------------------------------------------------------------------|---------------------|------|
| TNT                                                                                                   | percent             | 34.5 |
| Hexogen                                                                                               | do                  | 40.0 |
| Powdered aluminum                                                                                     | do                  | 25.0 |
| Calcium phosphate (spec. surface area 42 m. <sup>2</sup> /g.; bulk density 0.01 g./cm. <sup>3</sup> ) | do                  | 0.5  |
| Time                                                                                                  | seconds             | 46   |
| Specific weight                                                                                       | g./cm. <sup>3</sup> | 1.84 |
| Spot diameter                                                                                         | mm                  | 8.3  |

From this it is apparent that the addition of calcium phosphate according to the invention not only produces an excellent desensitizing effect and an obvious reduction of bleeding as compared with the conventional desensitizers, but also that the castings made from such compositions also have a greater specific weight than those made with the conventional desensitizers.

#### EXAMPLE 5

In the case of explosive compositions made from TNT (solidification point 80.47° C.) and tetryl (this two component mixture is known as tetrytol), the following spot diameters were measured and flashing or explosion occurred at 230° C. after the following periods—

#### Mixture A:

|               |         |    |
|---------------|---------|----|
| TNT           | percent | 30 |
| Tetryl        | do      | 70 |
| Time          | seconds | 28 |
| Spot diameter | mm      | 48 |

#### Mixture B:

|                                                                                                        |         |    |
|--------------------------------------------------------------------------------------------------------|---------|----|
| TNT                                                                                                    | percent | 30 |
| Tetryl                                                                                                 | do      | 69 |
| Calcium phosphate (spec. surface area 18 m. <sup>2</sup> /g.; bulk density 0.025 g./cm. <sup>3</sup> ) | do      | 1  |
| Time                                                                                                   | seconds | 42 |
| Spot diameter                                                                                          | mm      | 18 |

In these two experiments the explosive was not in powder form, but was placed in the test tube in the form of a piece weighing 0.4 g.

#### EXAMPLE 6

In the case of explosive compositions of TNT (solidification point 80.47° C.) and PETN (pentaerythritol tetrinitrate), flashing or explosion occurred at 230° C. after the periods of time specified hereinafter, and the spot diameters were as described—

#### Mixture A:

|                           |         |    |
|---------------------------|---------|----|
| TNT                       | percent | 50 |
| PETN                      | do      | 50 |
| Time                      | seconds | 27 |
| Spot diameter (at 65° C.) | mm      | 41 |

#### Mixture B:

|                                                                                                    |         |    |
|----------------------------------------------------------------------------------------------------|---------|----|
| TNT                                                                                                | percent | 50 |
| PETN                                                                                               | do      | 49 |
| Calcium phosphate (spec. surface area 20 m. <sup>2</sup> /g.; bulk density 0.02 cm. <sup>3</sup> ) | do      | 1  |
| Time                                                                                               | seconds | 34 |
| Spot diameter (at 65° C.)                                                                          | mm      | 13 |

In these two experiments the explosive was placed in the test tube not in powder form but in the form of a piece weighing 0.4 g.

## EXAMPLE 7

The following are the spot diameters and the time periods required to produce the flashing or explosion of explosive mixtures of tetryl, trinitrobenzene and hexogen at 230° C.—

## Mixture A:

|                 |         |    |
|-----------------|---------|----|
| Tetryl          | percent | 16 |
| Trinitrobenzene | do      | 24 |
| Hexogen         | do      | 60 |
| Time            | seconds | 30 |
| Spot diameter   | mm      | 50 |

## Mixture B:

|                                                                                                       |         |    |
|-------------------------------------------------------------------------------------------------------|---------|----|
| Tetryl                                                                                                | percent | 16 |
| Trinitrobenzene                                                                                       | do      | 24 |
| Hexogen                                                                                               | do      | 59 |
| Calcium phosphate (spec. surface area 15 m. <sup>2</sup> /g.; bulk density 0.03 g./cm. <sup>3</sup> ) | do      | 1  |
| Time                                                                                                  | seconds | 38 |
| Spot diameter                                                                                         | mm      | 19 |

The spot test was performed at 75° C. over a period of 2 hours.

## EXAMPLE 8

The addition of calcium phosphate to explosive compositions according to the invention can also be combined with the addition of other desensitizers. The desensitizing effect of such combined additives in this case can be increased considerably if, for example, a mixture of chlorinated naphthaline with a softening point of 116° C. is used as a desensitizer together with the calcium phosphate (spec. surf. area 15 m.<sup>2</sup>/g.; bulk density 0.03 g./cm.<sup>3</sup>). For explosive compositions made from tetryl and TNT (solidification point 80.47° C.), and known as tetrytol, the following are the spot diameters and the time periods required to produce flashing or explosion at 230° C.—

## Mixture A:

|                           |         |    |
|---------------------------|---------|----|
| Tetryl                    | percent | 70 |
| TNT                       | do      | 30 |
| Time                      | seconds | 28 |
| Spot diameter (at 60° C.) | mm      | 48 |

## Mixture B:

|                           |         |     |
|---------------------------|---------|-----|
| Tetryl                    | percent | 69  |
| TNT                       | do      | 30  |
| Chlorinated naphthaline   | do      | 1   |
| Time                      | seconds | 43  |
| Spot diameter (at 60° C.) | mm      | >50 |

## Mixture C:

|                           |         |    |
|---------------------------|---------|----|
| Tetryl                    | percent | 69 |
| TNT                       | do      | 30 |
| Calcium phosphate         | do      | 1  |
| Time                      | seconds | 42 |
| Spot diameter (at 60° C.) | mm      | 18 |

## Mixture D:

|                           |         |    |
|---------------------------|---------|----|
| Tetryl                    | percent | 68 |
| TNT                       | do      | 30 |
| Calcium phosphate         | do      | 1  |
| Chlorinated naphthaline   | do      | 1  |
| Time                      | seconds | 53 |
| Spot diameter (at 60° C.) | mm      | 20 |

In these 4 experiments the explosive was not placed in the test tube in powder form, but in the form of a piece weighing 0.4 g.

The specific surface area was measured according to Blaine's test. This test is described in the directives by the "Verein Deutscher Ingenieure" (VDI) (Association of German Engineers) No. 2031 of October 1962 under the title "Feinheitsbestimmungen an technischen Staubböden" and can be obtained from the VDI-Verlag GmbH, Düsseldorf, Germany.

What is claimed is:

1. In an explosive composition comprising fusible aromatic nitro compounds of the group trinitrotoluene and trinitrobenzene, the improvement which comprises calcium phosphate fume having a specific surface area of about 10–50 m.<sup>2</sup>/g. and a bulk density of about 0.01–0.07 g./cm.<sup>3</sup>, in a minor proportion effective to improve detonation characteristics, thermal stability or exudation characteristics.

2. Explosive composition according to claim 1, wherein the calcium phosphate fume is present in amount of about 0.1–15% by weight of the composition.

3. Explosive composition according to claim 2, said amount being about 0.2–5% by weight of the composition.

4. An explosive composition according to claim 1 containing a material of the group nitramines, nitric acid esters, and mixtures thereof.

5. An explosive composition according to claim 1 and containing metal powder.

## References Cited

## UNITED STATES PATENTS

3,271,212 9/1966 Riedl et al. 149—106 X

CARL D. QUARFORTH, Primary Examiner

S. J. LECHERT, Jr., Assistant Examiner

U.S. Cl. X.R.

149—39, 88, 92, 103, 105

UNITED STATES PATENT OFFICE  
CERTIFICATE OF CORRECTION

Patent No. 3,496,039 Dated Feb. 17, 1970

Inventor(s) Adolf Berthman, et al.

It is certified that error appears in the above-identified patent and that said Letters Patent are hereby corrected as shown below:

Col. 2, line 12, change "with" to --without--.

SIGNED AND  
SEALED

JUL 7 1970

(SEAL)

Attest:

Edward M. Fletcher, Jr.

Attesting Officer

WILLIAM E. SCUYLER, JR.  
Commissioner of Patents